

## UNITED STATES PATENT OFFICE

1,975,697

## PLASTICIZING ESTERS

Anthony M. Muckenfuss and Virgil L. Hansley,  
Niagara Falls, N. Y., assignors, by mesne assignments,  
to E. I. du Pont de Nemours and Company, a corporation of Delaware

No Drawing. Application March 19, 1932,  
Serial No. 600,061

18 Claims. (Cl. 106—37)

This invention relates to cellulose derivative compositions containing conditioners and more particularly to the use of certain esters derived from polycyclic hydrocarbons as conditioners in compositions such as those of nitrocellulose, cellulose acetate, and the like.

By the term "conditioner" we mean such materials as are added to the cellulosic compositions to modify their physical properties. Thus these 10 addition agents may be softeners or plasticizers; by this we mean that they may be of such low volatility, that is, having a boiling point of more than 200° C. at atmospheric pressure, that they remain in a film or other solid form formed from 15 the cellulosic bodies in which they are incorporated and impart flexibility and toughness thereto. A plasticizer is in general characterized as being a solvent for the cellulosic material in 20 which used, while a softener is not necessarily a solvent.

Various materials have heretofore been employed for these and analogous conditioning purposes; for example, castor oil and other vegetable oils, diphenylene phthalate, dibutyl phthalate 25 and other high boiling esters have variously been incorporated with cellulosic esters, such as nitrocellulose or cellulose acetate, for conditioning purposes.

One object of this invention is to provide new 30 and useful compositions of matter suitable for use as conditioners, e. g., plasticizers and/or softeners for cellulose ester compositions. A further object is to produce cellulosic compositions having particularly useful properties.

These objects may be accomplished by incorporating with suitable cellulose derivative compositions, esters derived from polycyclic hydrocarbons and more particularly, carboxylic acid esters derived from alkali metal compounds of 40 polycyclic hydrocarbons occurring in coal tar distillates and petroleum products e. g. a benzocyclopentadiene.

The invention will now be illustrated by esters derived from polycyclic hydrocarbons commonly 45 occurring in coal tar. The esters may be made from the pure hydrocarbons or from hydrocarbon mixtures, for instance coal tar distillates. Our method of preparing the esters consists in first reacting the hydrocarbon with alkali metal, reacting the resulting metal derivative with carbon dioxide to obtain a carboxylic acid salt and then esterifying by reacting the salt (a) with acid 50 and alcohol or (b) with alkyl halide. We have also prepared the esters by reacting the metal 55

derivatives with an alkyl halogen carbonate, for instance ethyl chlorocarbonate.

The following examples illustrate the preparation of typical esters derived from a benzo-cyclopentadiene.

*Example I.—Preparation of indene-3-carboxylic acid ethyl ester*

The indene cut of coal tar (boiling point of about 179–183° C.) is reacted with sodium, for 65 instance, by stirring 300 grams of indene with 34 grams of sodium at 110–112° C. for 2½ hours. The sodium is preferably added in two equal portions, the second portion of sodium being added when the first has completely reacted. The reaction is complete when gases cease to be evolved. The reaction is suitably carried out in an atmosphere inert to sodium in an autoclave or other closed vessel equipped with an agitator and an outlet for hydrogen gas. When the reaction is 75 completed, the sodium hydrocarbide, which analysis shows may be represented by the chemical formula:  $C_8H_7Na$ , separates as a viscous liquid layer.

This sodium hydrocarbide is converted into 80 the sodium salt of indene carboxylic acid by introducing  $CO_2$  at 60–120° C. with vigorous agitation until absorption of  $CO_2$  is complete as indicated by increased gas pressure.

The ester may be prepared from the sodium 85 salt by known methods, for instance by acidifying with hydrochloric or sulfuric acid and reacting with alcohol in the usual manner. The ethyl ester has a boiling point of 95–100° C. at a pressure of 1 mm. of mercury and boils at above 90 200° C. at atmospheric pressure.

*Example II.—The preparation of fluorene-9-carboxylic acid 2-butoxyethyl ester*

Fluorene may similarly be reacted with sodium 95 to produce sodium fluorene and thereafter reacted with  $CO_2$  to produce fluorene-9-carboxylic acid in a manner similar to that described for indene in Example I. The resulting sodium salt compound has according to analysis the formula: 100



By esterification of this salt with the monobutyl 105 ether of ethylene glycol in the presence of hydrochloric or sulfuric acid, the corresponding ester is obtained. This ester, which we term "fluorene-9-carboxylic acid 2-butoxyethyl ester", is a 110 colorless or light yellow liquid having a boiling

point of 295-300° C. at a pressure of 1 mm. of mercury and a specific gravity of 1.145. When cooled to -10° C., it becomes too viscous to stir but does not crystallize.

5 By the above described method we have prepared mono- and di-esters from a number of polycyclic hydrocarbons, including fluorene, indene, anthracene and naphthalene. We have discovered that such esters of polycyclic hydrocarbons have properties which make them excellent conditioners for cellulose derivative compositions. In addition to their high boiling points, they possess other properties which make them especially adapted for plasticizers and the like, for instance, they are in general solvents for both nitrocellulose and cellulose acetate and are miscible with most of the commonly used cellulose ester solvents.

20 In addition to the specific esters mentioned in Examples I and II, we have found the following esters of fluorene and indene to be especially effective as conditioners for nitrocellulose and cellulose acetate: fluorene - 9 - carboxylic acid methyl ester, fluorene-9-carboxylic acid ethyl ester, fluorene-9-carboxylic acid butyl ester, fluorene-9-carboxylic acid 2-methoxy ethyl ester, fluorene-9-carboxylic acid 2-ethoxy ethyl ester, fluorene - 9 - carboxylic acid 2 - phenylmethoxy ethyl ester, indene-3-carboxylic acid methyl ester.

25 Suitable compositions for producing a brushing lacquer are given in the following examples to further illustrate the invention.

### Example III

|                                                 | Grams |
|-------------------------------------------------|-------|
| Cellulose nitrate                               | 79    |
| Ethyl acetate                                   | 132   |
| Ethyl alcohol                                   | 79    |
| 40 Butyl acetate                                | 105   |
| Toluene                                         | 105   |
| Fluorene-9-carboxylic acid 2-butoxy ethyl ester | 50    |

45 On evaporation of the solvents in this mixture, a product is obtained which contains approximately 40% of the conditioning ester.

### Example IV

|                                      | Grams |
|--------------------------------------|-------|
| 50 Cellulose acetate                 | 80    |
| Acetone                              | 480   |
| Methyl cellosolve                    | 200   |
| Diacetone alcohol                    | 40    |
| Indene-3-carboxylic acid ethyl ester | 20    |

55 On evaporation of the solvents, the resulting product contains about 20% of the conditioning ester.

60 Films made by evaporation of solvents from compositions similar to those shown in Examples III and IV, containing from 20% to 65% by weight of polycyclic hydrocarbon carboxylic acid esters as conditioners, are homogeneous and transparent. The conditioners impart considerable toughness and plasticity to the films.

65 In place of a pure ester, a mixture of esters may be used as conditioner. Such a mixture may be obtained, for instance, by treating a coal tar or petroleum distillate containing several polycyclic hydrocarbons by the process illustrated by Examples I and II. A mixture of esters may sometimes also be made by similarly treating a pure hydrocarbon. For instance we have found that pure naphthalene yields a mixture of esters which probably contains isomers of naphthalene mono- and di-carboxylic acid esters.

The amounts of ester added as conditioner may be considerably varied. In general, the amount added to cellulose acetate will be lower than that permissible for nitrocellulose. It has been found that amounts ranging from 10-65% by weight of conditioner, determined in terms of the dried weight of the composition, give good results. 80

Our invention is not restricted to the specific examples given above and varying amounts of conditioners and other ingredients may be used without departing from the scope of the invention. 85

The compositions of the cellulosic material in which our conditioners are employed are subject to wide variations depending on whether one desires to produce thin films as in the case of a brushing lacquer, or relatively massive bodies, as in the case of the various molded articles made of pyroxylin. The invention is not restricted to specific compositions containing definite ratios of cellulose derivative to conditioner and/or solvent, nor to specific solvents. The usual experimentation which is within the province of one skilled in arts of this kind will of course be necessary in order to determine the optimum amounts 90 of conditioner, solvent, cellulose derivative, and other additions in the particular composition desired. Fillers and/or coloring bodies may be incorporated as desired. Stabilizers may also be added to the compositions in the usual amounts. 95

100 Among the advantages possessed by the conditioners of our invention are:

1. They are in general relatively good solvents for cellulose esters.
2. They are readily miscible with or dissolve many of the usual cellulose ester solvents.
3. They impart to cellulose ester compositions a high refractive index and a high resistance to moisture.
4. They do not lower the dielectric properties of the mixture to the extent of the now commonly used plasticizers.
5. They produce cellulose ester compositions which are of excellent toughness, homogeneity and plasticity.

105 We claim:

1. A composition of matter comprising a cellulose derivative, solvent therefor and conditioning amounts of an alkyl ester of a benzo-cyclopentadiene carboxylic acid.
2. A composition of matter comprising a cellulose derivative, a solvent therefor and a fluorene carboxylic acid alkyl ester.
3. A composition of matter comprising a cellulose derivative, a solvent therefor and an indene carboxylic acid alkyl ester.
4. A composition of matter comprising cellulose derivative, a solvent therefor and fluorene-9-carboxylic acid 2-butoxyethyl ester, the ratio of the weight of said ester to the weight of said cellulose derivative being from 1:9 to 13:7.
5. A composition of matter comprising cellulose derivative, a solvent therefor and indene-3-carboxylic acid ethyl ester, the ratio of the weight of said ester to the weight of said cellulose derivative being from 1:9 to 13:7.
6. A composition of matter comprising cellulose nitrate, a solvent therefor and a fluorene carboxylic acid alkyl ester.
7. A composition of matter comprising cellulose nitrate, a solvent therefor and an indene carboxylic acid alkyl ester.
8. A composition of matter comprising cellulose acetate, a solvent therefor and a fluorene carboxylic acid alkyl ester.

|     |                                                                                                                                                   |                                                                                                      |     |
|-----|---------------------------------------------------------------------------------------------------------------------------------------------------|------------------------------------------------------------------------------------------------------|-----|
| 9.  | A composition of matter comprising cellulose acetate, a solvent therefor and an indene carboxylic acid alkyl ester.                               | lose derivative, and 10-65% by weight of indene-3-carboxylic acid ethyl ester.                       |     |
| 10. | A composition of matter comprising a cellulose derivative, and conditioning amounts of an alkyl ester of a benzo-cyclopentadiene carboxylic acid. | 15. A composition of matter comprising cellulose nitrate and a fluorene carboxylic acid alkyl ester. | 80  |
| 11. | A composition of matter comprising a cellulose derivative and a fluorene carboxylic acid alkyl ester.                                             | 16. A composition of matter comprising cellulose nitrate, and an indene carboxylic acid alkyl ester. |     |
| 12. | A composition of matter comprising a cellulose derivative and an indene carboxylic acid alkyl ester.                                              | 17. A composition of matter comprising cellulose acetate and a fluorene carboxylic acid alkyl ester. | 85  |
| 13. | A composition of matter comprising cellulose derivative, and 10-65% by weight of fluorene-9-carboxylic acid-2-butoxyethyl ester.                  | 18. A composition of matter comprising cellulose acetate and an indene carboxylic acid alkyl ester.  |     |
| 14. | A composition of matter comprising cellulose derivative, and 10-65% by weight of fluorene-9-carboxylic acid-2-butoxyethyl ester.                  | ANTHONY M. MUCKENFUSS.<br>VIRGIL L. HANSLEY.                                                         | 90  |
| 20  |                                                                                                                                                   |                                                                                                      | 95  |
| 25  |                                                                                                                                                   |                                                                                                      | 100 |
| 30  |                                                                                                                                                   |                                                                                                      | 105 |
| 35  |                                                                                                                                                   |                                                                                                      | 110 |
| 40  |                                                                                                                                                   |                                                                                                      | 115 |
| 45  |                                                                                                                                                   |                                                                                                      | 120 |
| 50  |                                                                                                                                                   |                                                                                                      | 125 |
| 55  |                                                                                                                                                   |                                                                                                      | 130 |
| 60  |                                                                                                                                                   |                                                                                                      | 135 |
| 65  |                                                                                                                                                   |                                                                                                      | 140 |
| 70  |                                                                                                                                                   |                                                                                                      | 145 |
| 75  |                                                                                                                                                   |                                                                                                      | 150 |